# EUROPEAN PATENT SPECIFICATION

(11) **EP 2 430 206 B1**
(45) Date of publication and mention of the grant of the patent: **03.07.2013**
(21) Application number: 10711936.4
(22) Date of filing: 17.02.2010
(51) Int. Cl.: C23C 2/02, C23C 2/06, C23C 2/12, C23C 2/30

(54) **MODIFICATION OF THE COMPOSITION OF THE FLUX SOLUTION FOR HOT-DIP BATCH GALVANIZING OF STEEL PARTS**
VERÄNDERUNG DER ZUSAMMENSETZUNG EINER FLUSSMITTELLÖSUNG FÜR STÜCKFEUERVERZINKUNG VON STAHLTEILEN
MODIFICATION DE LA COMPOSITION DE LA SOLUTION DE FLUX POUR LA GALVANISATION EN LOTS PAR TREMPAGE À CHAUD DE PIÈCES D'ACIER

(30) Priority: 19.02.2009 IT AL20090002
(43) Date of publication of application: 21.03.2012
(73) Proprietor: SETRA SRL, 15121 Alessandria (IT)
(72) Inventor: BOTTANELLI, Ugo, I-15046 San Salvatore M.to (IT)
(74) Representative: Cinquantini, Bruno
(86) International application number: PCT/IT2010/000052
(87) International publication number: WO 2010/095154

(56) References cited:
- WO-A-2007/146161
- US-A1- 2006 228 482
- US-A1- 2007 137 731

## Description

The present invention has as object the improvement of the surface preparation of pre-fabricated steel parts to be hot-dip galvanized and more specifically it refers to the influence of the flux solution composition or the coating quality obtained in batch galvanizing processes where molten Zinc baths containing up to 0,1 wt% A1 are used.

The selection of the appropriate chemical solution composition together with special operating conditions, guarantee the satisfactory wetting of the steel part during the immersion into the molten Zn-afloy and an homogeneous and adherent coating.

### State of The Art

Batch hot-dip galvanizing is one of the most important technologies for steels coating against corrosion especially atmospheric. In this process steel parts are immersed into molten Zinc at 440-450°C. Even if improvements have been introduced for single operation in the industrial lines, the sequence of these operations are still the same since many years: a) degreasing followed by water rinsing, b) 10wt% HCl pickling followed by water rinsing, c) fluxing into a water-based saline solution which contains ZnC12+NH4Cl, followed by drying without rinsing, d) immersion into a molten Zn-based alloy at ≈440-450°C.

Steels that my be galvanized include those so-called: reactive. Steels reactivity depends on a critical concentration of Si and P in the steel (Sandelin effect) which may vary not only among the steels but also in the same steel where they may be unevenly distributed. Coatings obtained with reactive steels are gray and dull, the interface with the steel is fragile, the thickness of the coating is high causing excessive Zinc consumption and therefore an economical damage.

The fragile interface contains Zn-Fe phases that may reach the outer surface of the coating which due to its fragility may flake after a mechanical deformation.

The reason of this reactivity has not yet been thoroughly clarified even if many methods for its limitation have been proposed, based on the additions of metallic elements into the molten Zinc-bath, among which the most efficient are A1 and Ni.

Examples of these modification of the galvanizing baths composition are the so-called Polygalva based on 0.06wt% A1 addition, other methods based on less A1 additions, or the so-called Technigalva based on 0.05wt% ofNi addition.

It has been suggested also the addition of Sn=2.5%, Ni=0.05% or V=0.04%, Ti=0.05% which are claimed to be able to eliminate the Sandelin effect for steels containing up to Si≅ 1%. It has also proposed to add 1% Mn or 0.1-0.2% Mg.

The use of Aluminum additions to the Zinc bath has been studied for long time for its promising potentiality either for the inhibition of the interface Zn/Fe reaction either because its low cost compared to that of Ni.

Nevertheless its use has not been possible yet because in the actual process conditions, the presence of A1 in the bath causes defects such as not-coated areas which may reduce the corrosion resistance of the coated piece.

The solution for this problem is described in the Italian Patent RM2002A000589 and AL2008A000020 in which it is declaimed that by the use of a flux solution containing ZnCl₂ + NH₄Cl + BiCl₃ it is possible the use of Zn in which low amount of A1 may be added in order to obtain a significant reactivity reduction for the so-called reactive steel and coatings without surface defects.

Nevertheless this innovation does not take into account of the environmental restrictions introduced by the so-called Seveso law. In fact, in Italy, in the D.Lgs No. 65 dated March, 14, 2003 complying with the Directive 1999/45/CE & 2001/60/CE Art.6 Annex II, ZnCl2 is classified as dangerous toxic compound because may cause long-term adverse effects in the aquatic environment.

Its presence into the galvanizing shop has been therefore restricted and must be as low as possible.

The flux solution which traditionally contains a mixture of salts among which ZnCl2 is, according to its concentration, a potential source of danger for the environment and thus must be carefully monitored.

### Description of the invention

US 2007/0137731 and WO 2007/146161 disclose a flux for using in a hot dip galvanisation process containing e.g. 15-40 wt.% ZnCl2, 1-10 wt.% NH3CI, 1-6 wt.% KCI and more than 0.05 wt.% Bi2O3 and including an acidic component so that the flux has a pH of about 1.5 or less.

The present invention aims at contributing to the solution of potential problems arising from the presence of ZnCl2 in the galvanizing shop, by means of a procedure for the preparation of surface of pre-fabricated steel pieces to be hot-dip galvanized in a Zn-Al-alloy, according to which the concentration of ZnCl2 into the flux solution is maintained below the limit prescribed by the law and preferably down to zero.

According to this procedure, the steel pieces, after pickling are immersed into an aqueous solution containing: 0-50 g/L of ZnCl₂, preferably 0-25, and more preferably 0-10, 20-300 g/L of NH₄Cl, 0.1-1 g/L of Bi₂O₃, at a pH ranging from 0.1 e 1.5, preferably between 0.5 e 1, maintained in the optimum interval by means of HCl 0.1N or KOH 0.1N additions; pieces are immersed in the flux solution at a temperature between 4 and 50°C, preferably between 10 and 30°C and more preferably between 15 and 25°C, for an immersion time between 10s and 10 minutes, preferably between20s and 2 min. and more preferably between 30s and 1 min. After extraction from the flux solution, the steel pieces are dried at 60-120°C for a maximum time of 60 min.

The salts from the flux solution remain adherent to the steel pieces and have a fusion temperature well below the temperature of the molten galvanizing bath and are therefore easily eliminated upon immersion forming ashes and dross.

Using the flux solution according to the present invention it is possible to coat in a batch galvanizing bath containing a Zn-Al-afloy, both carbon and high strength steels. Also steels with high Si content, and/or Mn, and/or P (i.e. steels commercially known as Sandelin or Iper-sandelin steels), usually considered difficult steels for galvanizing for the excessive growth of the a fragile interface, may be easily coated using the flux solution according to the present invention obtaining coating with uniform thickness, with no surface defects and with a smooth surface without non-homogeneous areas.

### Some Preferred embodiments

The following Examples demonstrate certain preferred embodiments of the present invention, without in any way limiting the scope and objects of the invention.

Many hot-dip galvanizing experiments were made, with different flux mode and different galvanizing baths. Table 2 summarizes the obtained results.

Steels were processed according to the following procedure:
a. degreasing into an acidic aqueous commercial solution 10wt% concentrated, at room temperature for 10 minutes;
b. tap water rinsing;
c. HCl 10wt% pickling at room temp. for 15 minutes;
d. Tap water rinsing;
e. Fluxing according to Table 2;
f. Drying at 80°C in dry air;
g. Immersion into a molten Zn.0,03wt%Al at 450°C.

The following Table 1 contains the symbols with which the surface quality of coatings was assessed according its coating homogeneity & continuity, uniformity of the colour.

**Table 1.**

| Symbol | Merit |
|---|---|
| ■ | Very bad |
| | Bad |
| □ | Sufficient |
| ○ | Good |
| ⊙ | Excellent |

**Table 2**

| | FLUX | | | | | | | GALVANIZING | | |
|---|---|---|---|---|---|---|---|---|---|---|
| | ZnCl₂ | NH₄Cl | KOH | KCl | Bi³⁺ | Fe²⁺ | (pH) | Al in the molten bath | Immersion time | Merit |
| | g/L | g/L | g/L | g/L | g/L | g/L | | % | (s) | |
| Control | 138.00 | 144.00 | 95.35 | 63.00 | 0.52 | 3.49 | 1.2 | 0.02 | 180 | ○ |
| 1 | - | - | - | - | 0.50 | - | 1 | 5.00 | 60 | ■ |
| 2 | 0 | 50 | 75.68 | 50 | 0.50 | - | 1 | 5.00 | 60 | |
| 3 | 0 | 100 | 75.68 | 50 | 0.50 | - | 1 | 5.00 | 60 | □ |
| 4 | 25 | 100 | 75.68 | 50 | 0.50 | - | 1 | 5.00 | 60 | ○ |
| 5 | - | - | - | - | - | - | 8 (**) | 0.03 | 60 | ■ |
| 6 | - | - | - | - | - | - | 8 (**) | 0.03 | 180 | □ |
| 7 | - | - | - | - | - | - | 8 (**) | 0.03 | 180 (*) | ■ |
| 8 | - | - | - | - | 0.50 | - | 1 | 0.03 | 30 | ⊙ |
| 9 | - | - | - | - | 0.50 | - | 1 | 0.03 | 60 | ⊙ |
| 10 | - | - | - | - | 0.50 | - | 1 | 0.03 | 180 | ⊙ |
| 11 | - | - | - | - | 0.50 | - | 1 | 0.03 | 180 (*) | □ |
| 12 | 0 | 50 | 75.68 | 50 | 0.50 | - | 1 | 0.03 | 60 | ⊙ |
| 13 | 0 | 50 | 75.68 | 50 | 0.50 | - | 1 | 0.03 | 180 | ⊙ |
| 14 | 12 | 100 | 75.68 | 50 | 0.50 | - | 1 | 0.03 | 60 | ⊙ |
| 15 | 25 | 100 | 75.68 | 50 | 0.50 | - | 1 | 0.03 | 180 | ⊙ |
| 16 | 40 | 100 | 75.68 | 50 | 0.50 | - | 1 | 0.03 | 60 | ⊙ |
| 17 | 50 | 100 | 75.68 | 50 | 0.50 | - | 1 | 0.03 | 180 | ⊙ |

| | | | | | | | | | | |
|---|---|---|---|---|---|---|---|---|---|---|
| (*) specimes maintained for 1 hr in air after pickling and tap water rinsing (**) tap water rinsing | | | | | | | | | | |

## Claims

1. A batch hot-dip galvanizing process wherein steel parts are
(a) immersed, after pickling, into an aqueous flux solution, based on chlorides and further containing Bismuth oxide, said aqueous flux solution containing 0-50 g/I of ZnCl₂, 20-300 g/I of NH₄Cl, 0.1-1 g/l of Bi₂O₃, 10-100 g/I of KCI and having pH in a range between 0.1 and 1.5, maintained in said range by means of HCl or KOH 0.1 N additions, and a temperature between 4 and 50°C, the immersion time being between 10 seconds and 10 minutes;
(b) dried, after extraction from the aqueous flux solution, at 60 - 120°C for a maximum time of 60 minutes;
(c) hot-dip galvanized into an alloy containing mainly Zinc and 0.01wt% - 0.1wt% of Aluminum.

2. A process according to claim 1, wherein said aqueous flux solution contains 0-25 g/I of ZnCl₂, preferably 0-10 g/l.

3. A process according to claim 1, wherein before the step a) the steel parts are degreased into a commercial acidic aqueous 10wt% solution, at room temperature for 10 minutes; tap water rinsed; pickled into HCl 10wt% at room temperature for 15 minutes; again rinsed into tap water.

4. A process according to claim 3, wherein the pH is between 0.5 and 1 and the temperature is between 4 and 40°C.

5. A process according to claim 4, wherein the temperature is between 10 and 30°C, preferably between 15 and 25°C.

6. A process according to claim 3, wherein the pH is between 0.5 and 1 and the immersion time of steel parts is between 30 s and 2 min.

7. A process according to claim 6, wherein the immersion time of steel parts in the flux solution is between 20 s and 2 min.

8. A process according to claim 6, wherein the immersion time into the flux solution is between 30 s and 1 min.

## Patentansprüche

1. Chargen-Heißgalvanisierverfahren, bei dem Stahlteile
(a) nach Beizen, in eine wässrige Flussmittellösung basierend auf Chloriden und ferner enthaltend Bismuthoxid eingetaucht werden, wobei die wässrige Flussmittellösung 0 bis 50 g/l ZnCl₂, 20 bis 300 g/l NH₄Cl, 0,1 bis 1 g/l Bi₂O₃, 10 bis 100 g/l KCl enthält und einen pH-Wert in einem Bereich zwischen 0,1 und 1, 5, wobei der pH-Bereich mittels 0,1 N-HCl- oder 0,1 N-KOH-Zugaben aufrechterhalten wird, und eine Temperatur zwischen 4 und 50°C aufweist, wobei die Eintauchzeit zwischen 10 Sekunden und 10 Minuten beträgt,
(b) nach Extraktion der wässrigen Flussmittellösung bei 60 bis 120°C für eine maximale Zeit von 60 Minuten getrocknet werden,
(c) zu einer Legierung enthaltend hauptsächlich Zink und 0,01 Gew.-% bis 0,1 Gew.-% Aluminium feuergalvanisiert werden.

2. Verfahren nach Anspruch 1, wobei die wässrige Flussmittellösung 0 bis 25 g/l und vorzugsweise 0 bis 10 g/l ZnCl₂ enthält.

3. Verfahren nach Anspruch 1, wobei vor dem Schritt a) die Stahlteile in einer kommerziellen wässrigen 10 Gew.-%-Säure-Lösung bei Raumtemperatur für 10 Minuten entfettet werden, mit Leitungswasser gespült werden, in 10 Gew.-% HCl bei Raumtemperatur für 15 Minuten gebeizt werden und erneut mit Leitungswasser gespült werden.

4. Verfahren nach Anspruch 3, wobei der pH-Wert zwischen 0,5 und 1 beträgt und die Temperatur zwischen 4 und 40°C beträgt.

5. Verfahren nach Anspruch 4, wobei die Temperatur zwischen 10 und 30°C und vorzugsweise zwischen 15 und 25°C beträgt.

6. Verfahren nach Anspruch 3, wobei der pH-Wert zwischen 0,5 und 1 beträgt und die Eintauchzeit der Stahlteile zwischen 30 Sekunden und 2 Minuten beträgt.

7. Verfahren nach Anspruch 6, wobei die Eintauchzeit der Stahlteile in der Flussmittellösung zwischen 20 Sekunden und 2 Minuten beträgt.

8. Verfahren nach Anspruch 6, wobei die Eintauchzeit in der Flussmittellösung zwischen 30 Sekunden und 1 Minute beträgt.

## Revendications

1. Procédé discontinu de galvanisation à chaud par immersion dans lequel les pièces en acier sont
(a) immergées, après décapage, dans une solution de flux aqueuse, basée sur des chlorures et contenant en outre de l'oxyde de bismuth, ladite solution de flux aqueuse contenant 0-50 g/l de ZnCl₂, 20-300 g/l de NH₄Cl, 0, 1-1 g/l de Bi₂O₃, 10-100 g/l de KCl et ayant un pH dans une plage entre 0,1 et 1,5, maintenu dans ladite plage par ajouts de HCl ou de KOH à 0,1 N, et une température entre 4 et 50 °C, le temps d'immersion étant entre 10 secondes et 10 minutes ;
(b) séchées, après extraction hors de la solution de flux aqueuse, à 60-120 °C pendant une durée maximale de 60 minutes ;
(c) galvanisées à chaud par immersion dans un alliage contenant principalement du zinc et 0,01-0,1 % en poids d'aluminium.

2. Procédé selon la revendication 1, dans lequel ladite solution de flux aqueuse contient 0-25 g/l de ZnCl₂, de préférence, 0-10 g/l.

3. Procédé selon la revendication 1, dans lequel avant l'étape a) les pièces en acier sont dégraissées dans une solution acide commerciale aqueuse à 10 % en poids, à température ambiante pendant 10 minutes ; rincées à l'eau du robinet ; décapées dans du HCl à 10 % en poids à température ambiante pendant 15 minutes ; de nouveau rincées à l'eau du robinet.

4. Procédé selon la revendication 3, dans lequel le pH est entre 0,5 et 1 et la température est entre 4 et 40 °C.

5. Procédé selon la revendication 4, dans lequel la température est entre 10 et 30 °C, de préférence entre 15 et 25°C.

6. Procédé selon la revendication 3, dans lequel le pH est entre 0,5 et 1 et le temps d'immersion des pièces en acier est entre 30 s et 2 min.

7. Procédé selon la revendication 6, dans lequel le temps d'immersion des pièces en acier dans la solution de flux est entre 20 s et 2 min.

8. Procédé selon la revendication 6, dans lequel le temps d'immersion dans la solution de flux est entre 30 s et 1 min.
